

Feb. 28, 1933.

W. H. KLAR

1,899,200

CARVING MATERIAL

Filed April 20, 1931

*FIG. 1.*



*FIG. 2.*



*FIG. 3.*



*FIG. 4.*



INVENTOR.  
WALTER H. KLAR  
BY  
Chapin & Neal  
ATTORNEYS.

## UNITED STATES PATENT OFFICE

WALTER H. KLAR, OF SPRINGFIELD, MASSACHUSETTS, ASSIGNOR TO MILTON BRADLEY COMPANY, OF SPRINGFIELD, MASSACHUSETTS, A CORPORATION OF MASSACHUSETTS

## CARVING MATERIAL

Application filed April 20, 1931. Serial No. 531,506.

This invention relates to a new composite material suitable for being carved or sculptured into various forms and figured reliefs. It has for its object the provision of such a material as may be economically manufactured, and which will serve in place of real carving stone for practice carving and sculpture work in the home, schools and art centers.

10 The material most commonly used for such purposes heretofore has been ordinary hard soap, but soap in any of its commercial forms, while easy to cut and carve, is of a perishable nature and cannot be relied upon to maintain its shape or form in sculpture work because of its proneness to shrink as it dries out. My new material, on the other hand, will have all the advantages of soap as to its property of being easily cut and carved and will have 20 the further advantage of being non-shrinkable, more permanent in character and more nearly akin to a stone in its suitability for sculpture work.

My new material contains wax as one of its 25 constituents and may be molded or cast into blocks and slabs convenient for marketing and for special uses such as for cameo work and bas-reliefs. Likewise different slabs or pieces may be welded together for the fabrication 30 of architectural models and monumental sampling, and it will find various uses in games for children and in gift shop materials.

A further feature of the invention which 35 enhances its usefulness in the above fields is the possibility of its being made to simulate various types of marbles, the colors obtained ranging from white to black in all gradations, and in all types and colors from white Carrara to the travertine, including Vermont 40 greys, Georgia pinks, sienna browns and the like.

In the accompanying drawing:

Fig. 1 is a perspective view of an imitation 45 marble block for carving in the round; Fig. 2 is a similar view of a slab for bas-relief carving;

Fig. 3 is a transverse sectional view of a 50 cameo blank; and

Fig. 4 is a plan view of the blank shown in Fig. 3.

The material consists generally of a mixture of wax and filler, so compounded as to give the desired consistency, weight and high melting point. It may be colored in the process of manufacture to give a uniform characteristic appearance throughout the material.

In the production of a suitable embodiment of my invention as hereinafter specifically described, considerations of low cost and a desirable high melting point for the composition have dictated the choice of the wax materials, and in the selection of filler the simulation of a soft stone or the fibrous character of a wood have been considered.

A composition suitable for carving is formed of stearic acid, low melting paraffin (scale wax), hard wax, and a comminuted inert filler which may be lithopone, chalk, blanc fixe (barium sulphate), wood flour, asbestos, talc, or any other material of like nature. The use of wood flour or asbestos as the filler will give the composite material a fibrous character so that it may be carved and sawed like wood.

A useful form of my invention may be formed by the following materials in approximately the proportions specified.

|                                            |    |
|--------------------------------------------|----|
| 6 parts by weight of stearic acid          | 80 |
| 24 parts by weight of low melting paraffin |    |
| 1 part by weight of hard wax               |    |
| 75 parts by weight of terra alba.          |    |

In the foregoing formula, the stearic acid used has a melting point at approximately 128° F., the low melting paraffin at approximately 121° F., and the hard wax at approximately 215° F. The resulting mixture should have a melting point of 123° F. or somewhat higher, and the waxes should be chosen and proportioned to achieve this result so that the completed compound will not soften at any normal temperature. A relatively small proportion of the hard wax will suffice to provide this necessary high melting point for the mixture.

After melting the waxes they are incorporated with the filler, which has previously been warmed, by thorough mixing in a so-called Day mixer. When mixed, the whole is

taken out and the various colors, which may be natural oxides or permanent chemical colors, are very carefully stirred in so as to keep the character of the wax from becoming 5 muddy. The material is then poured into molds to give blocks such as shown at 1 in Fig. 1 or slabs 2 such as shown in Fig. 2. As shown at 3, the resulting blocks or slabs have a marbleized appearance and coloring and as indicated at 4 this characteristic appearance is 10 uniform throughout the material, rendering the material suitable for carving.

For cameo and similar work, the material is 15 poured into the mold in two (or more) layers 5 and 6, the layers being of different colors, to form blanks generally indicated at 7 of circular or other shape.

The specific composition above gives sufficient 20 resistance to cutting to permit fine accurate work with a sharp tool and will retain its shape under normal temperature conditions. It may be cut with a smooth wax-like 25 finish and is capable of taking a high degree of polish similar to a stove. A soft abrasive will polish it with a gloss, and a more rough abrasive can be used to produce an egg-shell finish for the surface.

It will be understood that some variation 30 may be made in the quantities of the material used to meet special conditions without departing from the scope of the invention.

What I claim is:

A material suitable for hand carving 35 formed substantially by weight of 6 parts stearic acid, 24 parts low melting paraffin, 1 part hard wax, and 75 parts terra alba.

In testimony whereof I have affixed my signature.

WALTER H. KLAR.

40

45

50

55

60

65